# EUROPEAN PATENT SPECIFICATION

(11) **EP 2 971 260 B1**
(45) Date of publication and mention of the grant of the patent: **19.06.2019**
(21) Application number: 14779082.8
(22) Date of filing: 07.03.2014
(51) Int. Cl.: C25C 1/10, C25B 11/04, C25B 11/12, C25B 15/02, C25B 1/21, C23C 18/24, C25D 5/56, C23C 18/20

(54) **ELECTROLYTIC GENERATION OF MANGANESE (III) IONS IN STRONG SULFURIC ACID**
ELEKTROLYTISCHE HERSTELLUNG VON MANGAN (III)-IONEN IN KONZENTRIERTER SCHWEFELSÄURE
PRODUCTION ÉLECTROLYTIQUE D'IONS MANGANÈSE (III) DANS DE L'ACIDE SULFURIQUE FORT

(30) Priority: 12.03.2013 US 201313795382
(43) Date of publication of application: 20.01.2016
(73) Proprietor: MacDermid Acumen, Inc., Waterbury, CT 06702 (US)
(72) Inventor: PEARSON, Trevor, Cradley Heath West Midlands B64 7HR (GB); CLARKE, Terence, Tettenhall Wolverhampton WV6 8TZ (GB); CHAPANERI, Roshan, V., Foleshill Coventry CV6 5JH (GB); ROBINSON, Craig, Coventry CV2 5LW (GB); HYSLOP, Alison, Great Barr Birmingham B43 5LW (GB); SINGH, Amrik, Coventry CV1 5HL (GB)
(74) Representative: Jenkins, Peter David
(86) International application number: PCT/US2014/021618
(87) International publication number: WO 2014/164272

(56) References cited:
- EP-A1- 2 025 708
- WO-A1-79/00258
- WO-A1-2006/054996
- WO-A2-2013/112268
- US-A- 4 170 527
- US-A- 4 279 705
- US-A- 5 213 665
- US-A- 5 213 665
- US-A- 5 246 553
- US-A1- 2003 024 821
- US-A1- 2010 155 255
- US-A1- 2011 140 035
- US-A1- 2011 140 035
- US-A1- 2012 045 680
- US-B1- 8 603 352
- CH COMNINELLIS ET AL: "Electrochemical production of manganic sulfate in concentrated H2SO4", JOURNAL OF THE ELECTROCHEMICAL SOCIETY, ELECTROCHEMICAL SOCIETY, INC, US, vol. 129, no. 4, April 1982 (1982-04), pages 749-752, XP002082878, ISSN: 0013-4651
- P. VAUDANO: "Oxydation d'alkyltoluène par le sulfate manganique préparé par électrochimie", CHIMIA, vol. 46, no. 4, April 1992 (1992-04), pages 103-106, XP9192297,

## Description

### FIELD OF THE INVENTION

The present invention relates generally to an improved process for etching platable plastics such as ABS and ABS/PC.

### BACKGROUND OF THE INVENTION

It is well known in the art to plate non-conductive substrates, (i.e. plastics) with metal for a variety of purposes. Plastic moldings are relatively inexpensive to produce and metal plated plastic is used for many applications. For example, metal plated plastics are used for decoration and for the fabrication of electronic devices. An example of a decorative use includes automobile parts such as trim. Examples of electronic uses include printed circuits, wherein metal plated in a selective pattern comprises the conductors of the printed circuit board, and metal plated plastics used for EMI shielding. ABS resins are the most commonly plated plastics for decorative purposes while phenolic and epoxy resins are the most commonly plated plastics for the fabrication of printed circuit boards.

Plating on plastic surfaces is used in the production of a variety of consumer items. Plastic moldings are relatively inexpensive to produce and plated plastic is used for many applications, including automotive trim. There are many stages involved in the plating of plastic. The first stage involves etching the plastic in order to provide mechanical adhesion of the subsequent metallic coatings and to provide a suitable surface for adsorption of the palladium catalyst which is typically applied in order to catalyze deposition of the initial metallic layer from an autocatalytic nickel or copper plating process. Following this, deposits of copper, nickel and/or chromium may be applied.

The initial etching of the plastic components is an essential part of the overall process. However, only certain types of plastic components are suitable for plating. The most common types of plastic for electroplating are acrylonitrile/butadiene/styrene (ABS) or a blend of ABS with polycarbonate (ABS/PC). ABS consists of two phases. The first phase is a relatively hard phase consisting of an acrylonitrile/styrene copolymer and the second phase is a softer polybutadiene phase.

Currently, this material is etched almost exclusively using a mixture of chromic and sulfuric acids, which is highly effective as an etchant for ABS and ABS/PC. The polybutadiene phase of the plastic contains double bonds in the polymer backbone, which are oxidized by the chromic acid, thus causing complete breakdown and dissolution of the polybutadiene phase exposed at the surface of the plastic which gives an effective etch to the surface of the plastic.

One problem with the traditional chromic acid etching step is that chromic acid is a recognized carcinogen and is increasingly regulated, requiring that wherever possible, the use of chromic acid is replaced with safer alternatives. The use of a chromic acid etchant also has well-known and serious drawbacks, including the toxicity of chromium compounds which makes their disposal difficult, chromic acid residues remaining on the polymer surface that inhibit electroless deposition, and the difficulty of rinsing chromic acid residues from the polymer surface following treatment. Additionally, hot hexavalent chromium sulfuric acid solutions are naturally hazardous to workers. Burns and upper respiratory bleeding are common in workers routinely involved with these chrome etch solutions. Thus, it is very desirable that safer alternatives to acidic chromium etching solutions be developed.

Early attempts to replace the use of chromic acid for etching plastics typically focused on the use of permanganate ions as an alternative to chromic acid. The use of permanganate in combination with acid is described in U.S. Patent No. 4,610,895 to Tubergen et al. Later, the use of permanganate in combination with an ionic palladium activation stage was suggested in U.S. Pat. Pub. No. 2005/019958 to Bengston. The use of acid permanganate solutions in combination with perhalo ions (e.g., perchlorate or periodate) was described in U.S. Pat. Pub. No. 2009/0092757 to Satou. Finally, the use of permanganate ions in the absence of alkali metal or alkaline earth metal cations was described in International Pub. No. WO 2009/023628 to Enthone.

Permanganate solutions are also described in U.S. Pat. No. 3,625,758 to Stahl et al.. Stahl suggests the suitability of either a chrome and sulfuric acid bath or a permanganate solution for preparing the surface. In addition, U.S. Pat. No. 4,948,630 to Courduvelis et al., describes a hot alkaline permanganate solution that also contains a material, such as sodium hypochlorite, that has an oxidation potential higher than the oxidation potential of the permanganate solution. U.S. Pat. No. 5,648,125 to Cane describes the use of an alkaline permanganate solution comprising potassium permanganate and sodium hydroxide, wherein the permanganate solution is maintained at an elevated temperature, i.e., between about 75°C to 93°C (165°F to 200°F).

As is readily seen, many etching solutions have been suggested as a replacement for chromic acid in processes for preparing non-conductive substrates for metallization. However, none of these processes have proven satisfactory for various economic, performance and/or environmental reasons and thus none of these processes have achieved commercial success or been accepted by the industry as a suitable replacement for chromic acid etching. In addition, the stability of these permanganate based etching solutions may also be poor, resulting in the formation of manganese dioxide sludge.

The tendency for permanganate based solutions to form sludge and undergo self-decomposition has been investigated by the inventors here. Under strongly acidic conditions, permanganate ions can react with hydrogen ions to produce manganese (II)

4MnO₄⁻ + 12H⁺ → 4Mn²⁺ + 6H₂O + 5O₂ (1)

The manganese(II) ions formed by this reaction can then undergo further reaction with permanganate ions forming a sludge of manganese dioxide according to the following reaction:

2MnO₄⁻ + 2H₂O + 3Mn²⁺ → 5MnO₂ + 4H⁺ (2)

Thus formulations based on strongly acidic permanganate solutions are intrinsically unstable irrespective of whether the permanganate ion is added by alkali metal salts of permanganate or is electrochemically generated *in situ.* In comparison to the currently used chromic acid etches, the poor chemical stability of acidic permanganate renders it effectively useless for large scale commercial application. Alkaline permanganate etches are more stable, and are widely used in the printed circuit board industry for etching epoxy based printed circuit boards, but alkaline permanganate is not an effective etchant for plastics such as ABS or ABS/PC. Thus, manganese (VII) is unlikely to gain widespread commercial acceptance as an etchant for these materials.

Attempts to etch ABS without the use of chromic acid have included the use of electrochemically generated silver (II) or cobalt (III). Certain metals can be anodically oxidized to oxidation states which are highly oxidizing. For example, cobalt can be oxidized from cobalt (II) to cobalt (III) and silver can be oxidized from silver (I) to silver (II).

However, there is currently no suitable commercially successful etchant for plastics based on either permanganate (in either acid or alkaline form), or manganese in any other oxidation state or by using other acids or oxidants.

Thus, there remains a need in the art for an improved etchant for preparing plastic substrates for subsequent electroplating that does not contain chromic acid and that is commercially acceptable.

### SUMMARY OF THE INVENTION

It is an object of the invention to provide an etchant for plastic substrates that does not contain chromic acid.

It is another object of the present invention to provide an etchant for plastic substrates that is commercially acceptable.

It is another object of the present invention to provide an etchant for plastic substrates that is based on manganese ions.

It is still another object of the present invention to provide an electrode that is suitable for use in a strong acid oxidizing electrolyte but that is not degraded by the electrolyte.

It is still another object of the present invention to provide a suitable electrode for the generation of manganese(III) ions in strong sulfuric acid that is commercially acceptable.

It is still another object of the present invention to provide an improved pretreatment step for conditioning the plastic substrate prior to etching.

In one embodiment, the present invention relates generally to an electrolytic cell comprising:
an electrolyte solution comprising manganese(III) ions in a solution of sulfuric acid and an additional acid selected from the group consisting of methane sulfonic acid, methane disulfonic acid and combinations thereof, wherein the solution comprises at least 8M sulfuric acid;
a cathode in contact with the electrolyte solution; and
an anode in contact with the electrolyte solution.

In another embodiment, the present invention relates generally to electrodes that are suitable for the electrochemical oxidation of manganese(II) ions to manganese(III) ions in a strong acid solution.

In another embodiment, the present invention relates generally to a method of electrochemical oxidation of manganese(II) ions to manganese(III) ions comprising the steps of:
providing an electrolyte comprising a solution of manganese(II) ions in a solution of sulfuric acid at a concentration of at least 8M, and an additional acid selected from the group consisting of methane sulfonic acid, methane disulfonic acid and combinations thereof in an electrolytic cell, wherein the electrolytic cell comprises an anode and a cathode;
applying a current between the anode and the cathode; and
oxidizing the electrolyte to form manganese(III) ions, wherein the manganese (III) ions form a metastable complex.

### DETAILED DESCRIPTION OF THE PREFERRED EMBODIMENTS

The inventors of the present invention have found that trivalent manganese can readily be produced by electrolysis at low current density of divalent manganese ions in a strong acid solution, preferably a strong sulfuric acid solution, most preferably an at least 8M sulfuric acid solution. More particularly, the inventors of the present invention have discovered that a solution of trivalent manganese ions in a strongly acidic solution is capable of etching ABS.

Trivalent manganese is unstable and is highly oxidizing (standard redox potential of 1.51 versus normal hydrogen electrode). In solution, it very rapidly disproportionates to manganese dioxide and divalent manganese via the following reaction:

2Mn³⁺ + 2H₂O → MnO₂ + Mn²⁺ + 4H+ (3)

However, in a strong sulfuric acid solution, the trivalent manganese ion becomes meta-stable and forms a cherry purple/red colored sulfate complex. The inventors have found that this sulfate complex is a suitable medium for the etching of ABS and has many advantages over chromium-free etches of the prior art.

Thus, a method of preparing a solution capable of etching a plastic substrate that is not claimed may be provided, the method comprising the steps of:
providing an electrolyte comprising a solution of manganese(II) ions in a solution of at least one acid in an electrolytic cell, wherein the electrolytic cell comprises an anode and a cathode; and
applying a current to the anode and cathode of the electrolytic cell; and
oxidizing the electrolyte to form manganese(III) ions, wherein the manganese (III) ions form a metastable complex.

In a preferred embodiment, the plastic substrate comprises ABS or ABS/PC.

While it is contemplated that both phosphoric acid and sulfuric acid would be suitable for compositions of the present invention, the acid is sulfuric acid. At ambient temperatures, the half life of the manganese(III) ions in 7M sulfuric acid is on of the order of 2 years. By comparison, the half-life of similar concentrations of manganese(III) ions in 7M phosphoric acid was around 12 days. It is suggested that the much higher stability of the manganese(III) ions in sulfuric acid is due to the formation of mangano-sulfate complexes and the higher concentration of available hydrogen ion concentration in the sulfuric acid solution. A further problem with the use of phosphoric acid is the limited solubility of manganese(III) phosphate. Thus, although other inorganic acids such as phosphoric acid can be usable in the compositions of the present invention, sulfuric acid is used.

The remarkable stability of manganese(III) ions in strong sulfuric acid provides the following advantages in use:
1) Because the Mn(III) ions are formed at a low current density, the power requirements for the process are typically very low.
2) Because the anode operates at a very low current density, a small cathode in relationship to the anode area can be used to prevent cathodic reduction of the Mn(III) ions. This obviates the need for a divided cell and makes the engineering of an etchant regeneration cell simpler.
3) Because the process does not produce permanganate ions, there is no possibility of producing manganese heptoxide in the solution (this is a considerable safety hazard as it is violently explosive).
4) Because of the high stability of the Mn(III) ions in strong sulfuric acid, the etchant can be sold ready for use. In production, the etchant requires only a small regeneration cell at the side of the tank in order to maintain the Mn(III) content of the etch and prevent the build-up of Mn(II) ions.
5) Because other etch processes are based on permanganate, the result of the reaction of permanganate with Mn(II) ions causes rapid "sludging" with manganese dioxide and a very short lifetime of the etch. This should not be an issue with the Mn(III) based etch (although there may be some disproportionation over time).
6) The electrolytic production of Mn(III) in accordance with the present invention does not produce any toxic gases. While some hydrogen may be produced at the cathode, owing to the low current requirements, this would be less than that produced by many plating processes.

As described herein, in a preferred embodiment the acid is sulfuric acid. The concentration of sulfuric acid is at least 8 molar, preferably between about 9 and about 15 molar. The concentration of sulfuric acid is important in the process. Below a concentration of about 9 molar, the rate of etch becomes slow and above about 14 molar, the solubility of manganese ions in the solution becomes low. Additionally, very high concentrations of sulfuric acid tend to absorb moisture from the air and are hazardous to handle. Thus, in a most preferred embodiment, the concentration of sulfuric acid is between about 12 and 13 molar, which is dilute enough to allow the safe addition of water to the etch and strong enough to optimize the etch rate of the plastic. At this concentration of sulfuric acid, up to around 0.08M of manganese sulfate can be dissolved at the preferred operating temperature of the etch. For optimal etching, the concentration of manganese ions in solution should be as high as it is feasible to achieve.

The manganese(II) ions are preferably selected from the group consisting of manganese sulfate, manganese carbonate and manganese hydroxide although other similar sources of manganese(II) ions known in the art would also be usable in the practice of the invention. The concentration of manganese(II) ions may be in the range of between about 0.005 molar up to saturation. In one embodiment, the electrolyte also comprises colloidal manganese dioxide. This may form to some extent as a natural result of disproportionation of manganese(III) in solution, or may be added deliberately.

Manganese(III) ions can be conveniently generated by electrochemical means by the oxidation of manganese(II) ions. In addition, it is generally preferable that the electrolyte not contain any permanganate ions.

As described herein, in order to obtain rapid rates of etching on the ABS plastic, it is necessary to use a high concentration of acid. The presence of sulfate or bisulfate ions is necessary to form a complex with the manganese ions and a molar concentration of sulfuric acid of at least 8M is necessary to obtain good stability of the etch. For good etching of plastic, it was found that a concentration of sulfuric acid of at least about 12M is necessary for rapid etching. This has the effect of reducing the solubility of manganese ions in the bath and the maximum solubility of manganese ions in the bath at operating temperature is about 0.08M. Because the etch rate depends on the concentration of manganese (III) ions in solution and the maximum conversion percentage to maintain stability is about 50%, it would be desirable to increase the amount of manganese which can be dissolved in the bath.

The inventors have found that it is possible to increase the amount of manganese that can be dissolved in the bath by replacing a portion of the sulfuric acid with another acid in which the manganese ions may be more soluble.

The choice of acids which may be suitable is limited. For example, hydrochloric acid would produce chlorine at the anodes and nitric acid would produce nitric oxides at the cathode. Perchloric and periodic acids would be expected to generate permanganate ions which would decompose to manganese dioxide. Organic acids would generally be rapidly oxidized by the manganese(III) ions. Thus, acids which would have both the necessary stability to oxidation and the ability to increase the solubility of manganese ions in the bath are methane sulfonic acid and methane disulfonic acid. Since the solubility of manganese(II) is much better in methane sulfonic acid (and sulfuric acid) than it is in methane disulfonic acid, the former choices produce better performance. Thus methane sulfonic acid is the preferred additional acid and sulfuric acid is the preferred primary acid.

Based thereon, the present invention also relates generally to an electrolyte for etching ABS and ABS/PC plastics comprising sulfuric acid in combination with either methane sulfonic acid or methane disulfonic acid in order to obtain better solubility of manganese ions in the bath, wherein the electrolyte contains at least 8M of sulfuric acid and contains about 0M to about 6M of methane sulfonic acid or methane disulfonic acid, preferably from about 1M to about 6M methane sulfonic acid.

More particularly, the present invention relates generally to an electrolytic cell comprising:
an electrolyte solution comprising manganese(III) ions in a solution of sulfuric acid and an additional acid selected from the group consisting of methane sulfonic acid, methane disulfonic acid and combinations thereof wherein the solution comprises at least 8M sulfuric acid;
a cathode in contact with the electrolyte solution; and
an anode in contact with the electrolyte solution.

In addition, the present invention also relates generally to a method of electrochemical oxidation of manganese(II) ions to manganese(III) ions comprising the steps of:
providing an electrolyte comprising a solution of manganese(II) ions in a solution of sulfuric acid at a concentration of at least 8M , and an additional acid selected from the group consisting of methane sulfonic acid, methane disulfonic acid and combinations thereof in an electrolytic cell wherein the electrolytic cell comprises an anode and a cathode;
applying a current between the anode and the cathode; and
oxidizing the electrolyte to form manganese(III) ions, wherein the manganese(III) ions form a metastable complex.

Once the electrolyte has been oxidized to form a metastable complex, the platable plastic may be immersed in the metastable complex for a period of time to etch the surface of the platable plastic. In one embodiment, the platable plastic is immersed in the metastable complex a temperature of between 30 and 80°C. The rate of etching increases with temperature and is slow below 50°C.

The upper limit of temperature is determined by the nature of the plastic being etched. ABS begins to distort above 70°C, thus in a preferred embodiment the temperature of the electrolyte is maintained between about 50 and about 70°C, especially when etching ABS materials. The time period of the immersion of the plastic in the electrolyte is preferably between about 10 to about 30 minutes.

Articles etched in this manner may be subsequently electroplated using conventional pretreatment for plated plastics or the etched surface of the plastic may be used to enhance the adhesion of paint, lacquers or other surface coatings.

The concentration of manganese(II) ions used in the etch of this invention can be determined by means of cyclic voltammetry. The oxidation is diffusion controlled so efficient agitation of the etch solution is necessary during the electrolytic oxidation process.

The anode and cathode usable in the electrolytic cell described herein may comprise various materials. The cathode may comprise a material selected from the group consisting of platinum, platinized titanium, niobium, iridium oxide coated titanium, and lead. In one preferred embodiment, the cathode comprises platinum or platinized titanium. In another preferred embodiment, the cathode comprises lead. The anode may also comprise platinized titanium, platinum, iridium/tantalum oxide, niobium, boron doped diamond, or any other suitable material.

The inventors discovered that while the combination of manganese(III) ions and strong sulfuric acid (i.e., 8-15 molar) can etch ABS plastic, the etchant is also very aggressive towards the electrodes necessary to produce the manganese(III) ions. In particular, anodes having a titanium substrate may be rapidly degraded by the etchant.

Therefore, in an attempt to determine a more suitable electrode material, various other electrode materials were examined, including lead and graphite. Vitreous carbon and reticulated vitreous carbon were determined to be more robust and were capable of producing manganese(III) ions when an electrical current, preferably of between 0.1 and 0.4 A/dm² (based on the nominal surface area), was applied. In addition, because vitreous carbon and reticulated vitreous carbon may not be cost-effective for use as the electrode in commercial applications, the anode may also be manufactured from woven carbon fiber.

Carbon fiber is manufactured from fibers of polyacrylonitrile (PAN). These fibers go through a process of oxidation at increasing temperatures followed by a carbonization step at a very higher temperature in an inert atmosphere. The carbon fibers are then woven into a sheet which is typically used in combination with various resin systems to produce high strength components. Carbon fiber sheets also have good electrical conductivity and the fibers typically have a turbostratic (i.e., disordered layer) structure. Without wishing to be bound by theory, it is believed that it is this structure which makes the carbon fibers effective as an electrode. The SP² hybridized carbon atoms in the lattice give good electrical conductivity while the SP³ hybridized carbon atoms link the graphitic layers together, locking them in place and thus providing good chemical resistance.

A preferred material for use in the electrodes of the invention comprises a woven carbon fiber containing at least 95% carbon and not impregnated with any resin. In order to facilitate the handling and the weaving process, carbon fibers are typically sized with an epoxy resin and this may comprise up to 2% of the fiber weight. At this low percentage, when used as an electrode, the epoxy sizing is rapidly removed by the high sulfuric acid content of the etch. This may cause an initial slight discoloration of the etch, but does not affect the performance. Following this initial "running in" stage, the anode appears to be resistant to the electrolyte and is effective at oxidizing manganese (II) ions to manganese(III).

Anodes can be constructed by mounting the woven carbon fiber material in a suitable frame with a provision made for electrical contact. It is also possible to use carbon fiber as a cathode in the generation of manganese(III) ions, but it is more convenient to use lead, particularly as the cathode is much smaller than the anode if an undivided cell is used.

The current density which can be applied in the electrolytic cell is limited in part by the oxygen overpotential on the anode material chosen. As an example, in the case of platinized titanium anodes, above a current density of approximately 0.4 A/dm², the potential of the anode is sufficiently high to liberate oxygen. At this point, the conversion efficiency of manganese(II) ions to manganese(III) ions falls and thus any further increase in current density is wasted. Furthermore, operating the anodes at the higher overpotential required to produce the higher current density tends to produce manganese dioxide at the anode surface rather than manganese(III) ions.

It was surprisingly discovered that lead anodes can be effectively used in the electrolytic cell described herein. Lead becomes passive in strong sulfuric acid due to the formation of a layer of lead sulfate on the surface which has very limited solubility in sulfuric acid. This renders the anode passive until a very high overpotential (More than 2V versus a standard hydrogen electrode) is reached. At potentials above this level, a mixture of oxygen and lead dioxide is produced. While, it would be expected that such a high operating potential would favor oxygen production and the formation of permanganate ions instead of manganese(III) ions, experiments using a lead anode produced only manganese(III) ions and no permanganate. This can be verified by diluting the etch with water - the manganese(III) ions disproportionate producing brown manganese dioxide and manganese(II) ions. Filtration of the solution produces a virtually colorless solution characteristic of manganese(II) ions rather than the purple color of permanganate ions.

The inventors of the present invention have discovered that monitoring the rate of oxidation is necessary when lead anodes are used because of the very high efficiency of these anodes for the oxidation of manganese(II) ions. Thus, if the rate of oxidation is not monitored and controlled, too high a proportion of the manganese(II) ions are oxidized, leaving a very low concentration of manganese(II). In the absence of manganese (II) ions, the anode begins to oxidize manganese (III) ions to manganese(IV), which rapidly forms insoluble manganese dioxide.

Based thereon, it is important that no more than 50%, and preferably no more than 25%, of the original concentration of manganese(II) ions be oxidized to manganese(III) ions in order to maintain the stability of the electrolyte. In the case of lead anodes, this involves monitoring the build-up of manganese(III) ions by titration of the etch solution or using a redox electrode and stopping the electrolysis when the manganese (III) content reaches the desired level. At a concentration of sulfuric acid of 12.5M, it is necessary to have a concentration of more than 0.01M of manganese(III) ions for effective etching and maximum stability, and no more than 0.04M based on a total manganese content of 0.08M.

The anodes may comprise lead or a suitable lead alloy, and the type of alloy chosen can affect the efficiency of conversion. Pure lead or lead containing a small percentage of tin are particularly effective and produce conversion efficiencies of approximately 70%. It was also discovered that with a reasonable degree of agitation, surprisingly high current densities can be applied and still maintain this conversion rate.

Upon prolonged electrolysis using a lead anode, it was observed that a film of manganese dioxide eventually formed. Once a significant amount of manganese dioxide has nucleated on the electrode surface, it tends to grow thicker quite quickly. However, manganese dioxide is readily reduced electrochemically back to manganese(II) ions. Thus, the accumulation of manganese dioxide can be mitigated or eliminated by the process of reversing the cell current periodically. The time period between current reversals is not critical as long as sufficient coulombic charge is applied during the reversal phase to reduce the amount of manganese dioxide which has deposited on the surface back to manganese(II) ions.

Based thereon, when using lead and lead alloy electrodes for the purpose of generating manganese(III) ions in sulfuric acid solutions for the purpose of etching ABS or ABS/PC, the electrolysis process is preferably interrupted when the manganese(III) ions have reached a suitable working concentration which may be between 0.01 and 0.04M based on a total manganese content of 0.08M, such that there remains in solution an effective amount of manganese(II) ions such that the bath is stable and does not precipitate excessive amounts of manganese dioxide. Preferred electrode materials include, for example, pure lead, lead antimony containing about 4% antimony, lead tin anodes containing up to 5% tin and lead/tin/calcium anodes. Other suitable lead alloys may also be used in the practice of the invention. In addition, the use of periodically reversed current prevents the build-up of manganese dioxide films on the anode. This is useful to maintain the conversion efficiency of the anodes and reduce or obviate the need to remove and clean the anodes from the etch tank or regeneration cell.

In addition, for efficient generation of manganese(III) ions, it is generally necessary to use an anode area which is large in comparison to the area of the cathode. Preferably, the area ratio of anode to cathode is at least about 10:1. By this means, the cathode can be immersed directly in the electrolyte and it is not necessary to have a divided cell. Although the process would work with a divided cell arrangement, this would introduce unnecessary complexity and expense.

The invention will now be illustrated with reference to the following non-limiting examples:

### Comparative Example 1:

A solution of 0.08 molar of manganese(II) sulfate in 12.5 molar sulfuric acid (500 ml) was heated to 70°C and a piece of platable grade ABS was immersed in the solution. Even after an hour immersed in this solution, there was no discernible etching of the test panel and upon rinsing, the surface was not "wetted" and would not support an unbroken film of water.

### Example 1:

The solution of Comparative Example 1 was electrolyzed by immersing a platinized titanium anode of an area of 1 dm² and a platinized titanium cathode of surface area 0.01 dm² in the solution and applying a current of 200 mA for 5 hours.

During this period of electrolysis, the solution was observed to change in color from almost colorless to a very deep purple/red color. It was confirmed that no permanganate ions were present.

This solution was then heated to 70°C and a piece of platable grade ABS was immersed in the solution. After 10 minutes of immersion, the test piece was fully wetted and would support an unbroken film of water after rinsing. After 20 minutes of immersion, the sample was rinsed in water, dried and examined using a scanning electron microscope (SEM). This examination revealed that the test piece was substantially etched and many etch pits were visible.

### Example 2:

A solution containing 12.5 M of sulfuric acid and 0.08 M manganese(II) sulfate was electrolyzed using a platinized titanium anode at a current density of 0.2 A/dm². A platinized titanium cathode having an area of less than 1% of the anode area was used in order to prevent cathodic reduction of the Mn(III) ions produced at the anode. The electrolysis was performed for long enough for sufficient coulombs to be passed to oxidize all of the manganese(II) ions to manganese(III). The resulting solution was a deep cherry purple/red color. There were no permanganate ions generated during this step. This was also confirmed by visible spectroscopy - the Mn(III) ions produced a completely different absorption spectrum from that of a solution of permanganate.

### Example 3:

The etching solution prepared as described above in Example 2 was heated to 65-70°C on a magnetic stirrer/hotplate and test coupons of ABS were immersed in the solution for time periods of 20 and 30 minutes. Some of these test coupons were examined by SEM and some were processed in a normal plating on plastic pretreatment sequence (reduction in M-neutralize, predip, activate, accelerate, electroless nickel, copper plate to 25- 30 microns). These test coupons were then annealed and subjected to peel strength testing using an Instron machine.

Peel strength testing carried out on coupons plated for 30 minutes demonstrated peel strength varying between about 1.5 and 4 N/cm.

Cyclic voltammograms were obtained from a solution containing 12.5M sulfuric acid and 0.08M manganese sulfate using a platinum rotating disk electrode (RDE) having a surface area of 0.196 cm² at various rotation speeds. A model 263A potentiostat and a silver/silver chloride reference electrode were used in conjunction with the RDE.

In all cases, the forward scan showed a peak at around 1.6V vs. Ag/AgCl followed by a plateau up to around 1.75V followed by an increase in current. The reverse scan produced a similar plateau (at a slightly lower current and a peak around 1.52V. The dependence of these results on the rate of electrode rotation indicates mass transport control is a primary factor in the mechanism. The plateau indicates the potential range over which Mn(III) ions are formed by electrochemical oxidation.

A potentiostatic scan was performed at 1.7V. It was observed that the current initially dropped and then over a period of time increased. The current density at this potential varied between 0.15 and 0.4 A/dm².

Following this experiment, a galvanostatic measurement was taken at a constant current density of 0.3 A/dm². Initially, the applied current density was achieved by a potential of about 1.5V but as the experiment progressed, after about 2400 seconds, and increase in potential to about 1.75V was observed.

After a period of etching for more than 10 minutes, it was observed that the surface of the ABS test coupons was fully wetted and would support an unbroken film of water after rinsing. After a period of 20 or 30 minutes, the panels were noticeably etched.

### Example 4:

A solution was formulated comprising 10.5M sulfuric acid and 2M methane sulfonic acid. At a temperature of 68-70°C, it was possible to dissolve 0.16M of manganous sulfate with ease, whereas in the comparative case of dissolving manganous sulfate in a solution of 12.5M sulfuric acid, it was only possible to dissolve 0.08M. The formulated solution was electrolyzed to produce a manganese(III) concentration of 0.015M manganese(III) ions, which gave a comparable etch rate to that obtained from a solution of 12.5M sulfuric acid having a manganese(III) concentration of 0.015M.

Electrolysis was continued in the bath of Example 4 until the manganese(III) content reached 0.04M and another panel was etched. An enhanced etch rate was obtained at this higher concentration of manganese(III) ions (approximately 25% higher than that obtained at a concentration of 0.015M).

### Comparative Example 2:

An electrode comprising graphite and having a nominal measured surface area of 1 dm² was immersed in 500 mL of a solution containing 0.08 M of manganese sulfate in 12.5 M sulfuric acid at a temperature of 65°C. The cathode in this cell was a piece of lead having a nominal measured surface area of 0.1 dm². A current of 0.25 amps was applied to the cell, giving a nominal anode current density of 0.25 A/dm² and a nominal cathode current density of 2.5 A/dm².

It was observed that the graphite anode rapidly crumbled and degraded within less than 1 hour of electrolysis. In addition, no oxidation of manganese(II) ions to manganese(III) was observed.

### Comparative Example 3:

An electrode comprising a titanium substrate coating with a mixed tantalum/iridium oxide coating (50% tantalum oxide, 50% iridium oxide) and having a nominal measured surface area of 1 dm² was immersed in 500 mL of a solution containing 0.08 M of manganese sulfate in 12.5 M sulfuric acid at a temperature of 65°C. The cathode in this cell was a piece of lead having a nominal measured surface are of 0.1 dm². A current of 0.25 amps was applied to the cell giving a nominal anode current density of 0.25 A/dm² and a nominal cathode current density of 2.5 A/dm².

It was observed that manganese(III) was rapidly formed in the solution and the resulting solution was capable of etching ABS plastic and producing good adhesion upon subsequent electroplating of the treated plastic. However, after a period of two weeks operation (electrolyzing the solution for 8 hours/day), it was observed that the coating was lifting from the titanium substrate and that the titanium substrate itself was dissolving in the solution.

### Comparative Example 4:

An electrode comprising a titanium substrate coated with platinum and having a nominal measured surface area of 1 dm² was immersed in 500 mL of a solution containing 0.08 M of manganese sulfate in 12.5 M sulfuric acid at a temperature of 65°C. The cathode in this cell was a piece of lead having a nominal measured surface area of 0.1 dm². A current of 0.25 amps was applied to the cell giving a nominal anode current density of 0.25 A/dm² and a nominal cathode current density of 2.5 A/dm².

It was observed that manganese(III) was rapidly formed in the solution and the resulting solution was capable of etching ABS plastic and producing good adhesion upon subsequent electroplating of the treated plastic. However, after a period of two weeks operation (electrolyzing the solution for 8 hours/day), it was observed that the coating was lifting from the titanium substrate and that the titanium substrate itself was dissolving in the solution.

### Example 5:

An electrode comprising vitreous carbon and having a nominal measured surface area of 0.125 dm2 was immersed in 100 mL of a solution containing 0.08 M of manganese sulfate in 12.5 M sulfuric acid at a temperature of 65°C. The cathode in this cell was a piece of platinum wire having a nominal measured surface area of 0.0125 dm². A current of 0.031 amps was applied to the cell giving a nominal anode current density of 0.25 A/dm² and a nominal cathode current density of 2.5 A/dm².

It was observed that manganese(III) was rapidly formed in the solution and the resulting solution was capable of etching ABS plastic and producing good adhesion upon subsequently electroplating the treated plastic. The electrode appeared unaffected by periods of extended electrolysis.

### Example 6:

An electrode comprising a piece of woven carbon fiber (Panex 35 50K Tow with epoxy sizing at 1.5%, available from the Zoltek Corporation) was mounted in a plastic frame constructed of polyvinylidenefluoride (PVDF). The electrode, having a nominal measured area of 1 dm², was immersed in 500 mL of a solution containing 0.08 M of manganese sulfate in 12.5 M sulfuric acid at a temperature of 65°C. The cathode in this cell was a piece of lead having a nominal measured surface area of 0.1 dm². A current of 0.25 amps was applied to the cell, giving a nominal anode current density of 0.25 A/dm² and a nominal cathode current density of 2.5 A/dm².

It was observed that manganese(III) was rapidly formed in the solution and the resulting solution was capable of etching ABS plastic and producing good adhesion upon subsequent electroplating of the treated plastic. The electrode appeared unaffected by periods of extended electrolysis. Electrolysis was carried out over two weeks using this electrode and no observable degradation could be detected. The low cost and ready availability of this material makes it suitable for many commercial applications.

### Example 7:

An anode consisting of lead having an effective surface area (i.e., not counting the back of the electrode) of 0.4 dm² was immersed in a beaker containing 2 liters of a solution comprising 0.08M of manganese sulfate in 12.5M sulfuric acid at a temperature of 68-70°C. The other electrode in the cell consisted of a lead cathode having a surface area of approximately 0.04 dm². The solution was stirred using a magnetic stirrer to obtain moderate agitation over the surface of the electrolyte. A current density of 0.4 A/dm² was applied to the anode and the rate of manganese(III) was determined versus electrolysis time. The amount of manganese(III) was determined by diluting a sample of the bath with phosphoric acid to prevent disproportionation of the manganese(III) and titrating with a solution of ferrous ammonium sulfate using diphenylamine dissolved in acid as an indicator.

The experiment was repeated using a current density of 0.8 A/dm² and 1.6 A/dm². Under the hydrodynamic conditions of the experiment (i.e., moderate agitation using a magnetic stirrer), the oxidation did not appear to be mass transport limited at a current density of 1.6 A/dm² as the conversion efficiency was the same as that obtained at 0.4 A/dm² (70%). A further experiment was conducted at 3.2 A/dm² and it was found that the conversion efficiency had fallen to 42% and the rate of manganese(III) generation was only about 10% higher than that obtained at 1.6 A/dm². This indicates that under the agitation conditions used in the experiment, the overall limiting current density for manganese generation was about 1.6 A/dm². This corresponds to a conversion rate approximately four times higher than that which can be achieved from a platinized titanium anode.

The results of these experiments demonstrate that manganese(III) ions can be generated by electrosynthesis using manganese(II) ions in sulfuric acid at a relatively high concentration and operating at low current densities using a platinum or platinized titanium anode and that further improvements to the process can be realized by using various other anode materials, including vitreous carbon, carbon fiber, lead and lead alloy anodes.

Furthermore, the slower etch rate of the manganese based etch of the invention as compared with the etch rate obtained from a chromic acid etch has demonstrated a need to provide a pretreatment step to produce higher adhesion values and enable shorter etch times.

The aim of the pretreatment step is to condition the surface of the plastic to be etched so that it is etched more rapidly and evenly, leading to shorter etch times and better adhesion.

The use of solvents to condition the surface of ABS plastics is known. However, recent regulations strictly limit the viability of using volatile solvents on a plating line as they are often flammable and have health and safety issues (many are reprotoxic and may also cause liver damage). Thus, the choice of solvents is limited.

Propylene carbonate is a relatively safe solvent having good water solubility, low toxicity and low flammability (flash point is 135°C) and is ideal from a health and safety point of view. Gamma butyrolactone also works but is more toxic and in some countries is a controlled drug due to its recreational use.

In the present invention it was discovered that better results may be obtained in combination with the manganese based etch solutions described herein when the use of propylene carbonate is combined with an organic hydroxy acid such as lactic acid, glycolic acid or gluconic acid. The use of propylene carbonate on its own or with a wetting agent gives good adhesion and reduced etch times, but the cosmetic appearance of ABS/PC blends is poor after etching, activation and subsequent plating because it is prone to pitting. The combination of propylene carbonate with these hydroxy acids in the pretreatment stage is effective in preventing this problem.

Typically, the concentration of propylene carbonate is between about 100 and about 500 mL/L and the concentration of the organic acid is between about 100 and about 500 mL/L. In addition, the operating temperature is typically between about 20° and 70°C and the immersion time is between about 2 and about 10 minutes.

Thus, the present invention also relates generally to a pretreatment composition for the platable plastic substrate comprising Gamma butyrolactone or propylene carbonate in combination with an organic hydroxy acid such as lactic acid, glycolic acid or gluconic acid.

### Comparative Example 5:

A test coupon composed of an ABS/PC blend consisting of 45% polycarbonate was immersed in a solution containing 150 mL/L of propylene carbonates for the times and temperature shown in Table 1. Following this, the panel was rinsed and etched in a solution containing 12.5M sulfuric acid and 0.08M manganese, where 0.015M of the manganese ions had been electrolytically oxidized to manganese(III). The etching was carried out for 30 minutes at a temperature of 68-70°C. Following this treatment, the panel was rinsed, activated using a standard plating on plastics pretreatment sequence (MacDermid D34 palladium activator, MacDermid accelerator and MacDermid J64 electroless nickel in accordance with the technical data sheets) and then electroplated in copper. The cosmetic appearance of the panels was examined and a quantitative adhesion test was performed by pulling off the deposit from the substrate using an Instron tensile testing machine. The adhesion values obtained are shown in Table 1.

**Table 1. Adhesion values**

| | **Adhesion (N/cm)** | | |
|---|---|---|---|
| | **Side 1** | **Side 2** | **Average** |
| 10 minutes, 40°C | 8.46 | 9.23 | 8.85 |
| 5 minutes, 40°C | 4.78 | 5.19 | 4.99 |
| 10 minutes, 70°C | 5.79 | 5.02 | 5.41 |
| 5 minutes, 70°C | 11.54 | 8.77 | 10.16 |

The adhesion values are quite variable and it was noted that spots and pitting were observed on the plated parts. The copper coating was also pitted.

### Example 8:

The experiments performed in Comparative Example 5 were repeated but using a pre-conditioner comprising 150 mL/L of propylene carbonate and 250 mL/L of 88% lactic acid solution. These results of these tests are shown in Table 2.

**Table 2. Adhesion values**

| | **Adhesion (N/cm)** | | |
|---|---|---|---|
| | **Side 1** | **Side 2** | **Average** |
| 10 minutes, 40°C | 9.75 | 7.55 | 8.65 |
| 5 minutes, 40°C | 9.84 | - | 9.84 |
| 10 minutes, 70°C | 9.32 | 9.61 | 9.47 |
| 5 minutes, 70°C | 9.17 | 10.03 | 9.60 |

Using this preconditioner, which included the lactic acid, gave improvements in the consistency of adhesion. After plating, it was noted that the cosmetic appearance was excellent, being free of spots and pitting.

## Claims

1. An electrolytic cell comprising:
an electrolyte solution comprising manganese(III) ions and manganese(II) ions in a solution of comprising sulfuric acid and an additional acid selected from the group consisting of methane sulfonic acid, methane disulfonic acid and combinations thereof, wherein the solution comprises at least 8M sulfuric acid;
a cathode in contact with the electrolyte solution; and
an anode in contact with the electrolyte solution.

2. The electrolytic cell according to claim 1, wherein the solution optionally comprises at least 12M sulfuric acid, and/or
wherein the solution comprises between 1M and 6M methane sulfonic acid or methane disulfonic acid, and/or
wherein the solution comprises from 9 to 15 molar sulfuric acid and between 1M and 6M methane sulfonic acid.

3. The electrolytic cell according to claim 1, wherein an area of the anode is larger than an area of the cathode and/or wherein the anode comprises a material selected from the group consisting of vitreous carbon, reticulated vitreous carbon, woven carbon fibers, lead, lead alloy, platinized titanium, platinum, iridium/tantalum oxide, niobium, boron doped diamond, and combinations of one or more of the foregoing, preferably lead or lead alloy;
wherein when the anode comprises lead or lead alloy, the electrolytic cell also optionally comprises a means for monitoring the concentration of Mn(II) in the solution.

4. The electrolytic cell according to claim 1, wherein the cathode comprises a material selected from the group consisting of platinum, platinized titanium, iridium/tantalum oxide, niobium and lead,
optionally wherein the cathode comprises lead or
wherein the cathode comprises platinized titanium or platinum.

5. A method of electrochemical oxidation of manganese(II) ions to manganese(III) ions comprising the steps of:
providing an electrolyte comprising a solution of manganese(II) ions in a solution of sulfuric acid at a concentration of at least 8M , and an additional acid selected from the group consisting of methane sulfonic acid, methane disulfonic acid and combinations thereof in an electrolytic cell, wherein the electrolytic cell comprises an anode and a cathode;
applying a current between the anode and the cathode; and
oxidizing the electrolyte to form manganese(III) ions, wherein the manganese(III) ions form a metastable complex.

6. The method according to claim 5, wherein the electrolyte comprises between 1M and 6M methane sulfonic acid.

7. The method according to claim 5, wherein the anode comprises lead or lead alloy,
optionally further comprising the step of monitoring the buildup of manganese(III) ions in the solution;
further optionally wherein when the method comprises the step of monitoring the buildup of manganese(III) ions in the solution, optionally no more than 50% of the original concentration of manganese(II) ions is oxidized to manganese(III) ions, preferably no more than 25% of the original concentration of manganese(II) ions is oxidized to manganese(III) ions; and/or
further optionally wherein when the method comprises the step of monitoring the buildup of manganese(III) ions in the solution, the buildup of manganese(III) ions is optionally monitored using a redox electrode, wherein electrolysis is stopped when the manganese(III) content reaches the desired level; and/or
further optionally wherein when the method comprises the step of monitoring the buildup of manganese(III) ions in the solution, the buildup of manganese(III) ions is optionally monitored by titrating the etch solution, wherein electrolysis is stopped when the manganese(III) content reaches the desired level; and/or
further optionally wherein when the method comprises the step of monitoring the buildup of manganese(III) ions in the solution, the method further comprises monitoring the concentration of manganese(II) ions in the solution.

8. The method according to claim 5, comprising the step of periodically reversing the current in the electrolytic cell, whereby buildup of manganese dioxide on the anode is prevented.

9. The method according to claim 5, further comprising the step of contacting a platable plastic with the metastable complex for a period of time to etch the platable plastic,
optionally wherein the platable plastic comprises acrylonitrile-butadiene-styrene or acrylonitrile-butadiene-styrene/polycarbonate, and/or
wherein prior to contacting the platable plastic with the metastable complex, the platable plastic is contacted with a pretreatment composition to condition the surface of the platable plastic, the pretreatment composition comprising a solvent selected from the group consisting of propylene carbonate, gamma butyrolactone, and combinations thereof, preferably wherein the solvent comprises propylene carbonate,
optionally wherein the pretreatment solution further comprises an organic hydroxy acid, preferably wherein the organic hydroxy acid is selected from the group consisting of lactic acid, glycolic acid, gluconic acid and combinations of one or more of the foregoing;
further optionally wherein when the pretreatment solution comprises an organic hydroxy acid, the pretreatment composition is maintained at a temperature of between 20 to 70°C and the platable plastic is contacted with the pretreatment composition for 2 to 10 minutes.

10. The method according to claim 5, wherein the manganese (II) ions are derived from a compound selected from the group consisting of manganese sulfate, manganese carbonate and manganese hydroxide, and/or
wherein the solution additionally comprises colloidal manganese dioxide, and/or
wherein the concentration of the manganese (II) ions in the electrolyte is between 0.005 molar and saturation, and/or
wherein the electrolyte does not contain any permanganate.

11. The method according to claim 5, wherein the cathode comprises a material selected from the group consisting of platinum, platinized titanium, iridium/tantalum oxide, niobium and lead,
optionally wherein the cathode comprises lead and/or
wherein the cathode comprises platinized titanium or platinum.

12. The method according to claim 5, wherein the anode current density is between 0.1 to 0.4 A/dm², and/or
wherein the temperature of the electrolyte is maintained between 30°C and 80°C.

## Patentansprüche

1. Elektrolytische Zelle, umfassend:
eine Elektrolytlösung, die Mangan(III)-Ionen und Mangan(II)Ionen in einer Lösung umfasst, die Schwefelsäure und eine zusätzliche Säure umfasst, die aus der Gruppe bestehend aus Methansulfonsäure, Methandisulfonsäure und Kombinationen davon ausgewählt ist, wobei die Lösung mindestens 8M Schwefelsäure umfasst;
eine Kathode in Kontakt mit der Elektrolytlösung und
eine Anode in Kontakt mit der Elektrolytlösung.

2. Elektrolytische Zelle nach Anspruch 1, wobei die Lösung optional mindestens 12M Schwefelsäure umfasst und/oder:
wobei die Lösung zwischen 1M und 6M Methansulfonsäure oder Methandisulfonsäure umfasst und/oder
wobei die Lösung von 9 bis 15 Mol Schwefelsäure und zwischen 1M und 6M Methansulfonsäure umfasst.

3. Elektrolytische Zelle nach Anspruch 1, wobei eine Fläche der Anode größer als eine Fläche der Kathode ist und/oder wobei die Anode ein Material umfasst, das aus der Gruppe bestehend aus Glaskohlenstoff, netzartigem Glaskohlenstoff, Kohlenstofffasergewebe, Blei, Bleilegierung, platiniertem Titan, Platin, Iridium-/Tantaloxid, Niob, bordotiertem Diamant und Kombinationen von einem oder mehreren der vorstehenden ausgewählt ist, vorzugsweise Blei oder Bleilegierung ist;
wobei, wenn die Anode Blei oder Bleilegierung umfasst, die elektrolytische Zelle außerdem optional ein Mittel zum Überwachen der Konzentration von Mn(II) in der Lösung umfasst.

4. Elektrolytische Zelle nach Anspruch 1, wobei die Kathode ein Material umfasst, das aus der Gruppe bestehend aus Platin, platiniertem Titan, Iridium-/Tantaloxid, Niob und Blei ausgewählt ist,
optional wobei die Kathode Blei umfasst oder
wobei die Kathode platiniertes Titan oder Platin umfasst.

5. Verfahren zur elektrochemischen Oxidation von Mangan(II)-Ionen zu Mangan(III)-Ionen, das die folgenden Schritte umfasst:
Bereitstellen eines Elektrolyts, der eine Lösung von Mangan(II)-Ionen in einer Lösung von Schwefelsäure mit einer Konzentration von mindestens 8M und einer zusätzlichen Säure, die aus der Gruppe bestehend aus Methansulfonsäure, Methandisulfonsäure und Kombinationen davon ausgewählt ist, umfasst, in einer elektrolytischen Zelle, wobei die elektrolytische Zelle eine Anode und eine Kathode umfasst;
Anlegen eines Stroms zwischen der Anode und der Kathode und
Oxidieren des Elektrolyts, um Mangan(III)-Ionen zu bilden, wobei die Mangan(III)-Ionen einen metastabilen Komplex bilden.

6. Verfahren nach Anspruch 5, wobei der Elektrolyt zwischen 1M und 6M Methansulfonsäure umfasst.

7. Verfahren nach Anspruch 5, wobei die Anode Blei oder Bleilegierung umfasst,
das optional weiterhin den Schritt eines Überwachens der Ansammlung von Mangan(III)-Ionen in der Lösung umfasst;
weiterhin optional wobei, wenn das Verfahren den Schritt des Überwachens der Ansammlung von Mangan(III)-Ionen in der Lösung umfasst, optional nicht mehr als 50 % der ursprünglichen Konzentration von Mangan(II)-Ionen zu Mangan(III)-Ionen oxidiert wird, vorzugsweise nicht mehr als 25 % der ursprünglichen Konzentration von Mangan(II)-Ionen zu Mangan(III)-Ionen oxidiert wird; und/oder
weiterhin optional wobei, wenn das Verfahren den Schritt des Überwachens der Ansammlung von Mangan(III)-Ionen in der Lösung umfasst, die Ansammlung von Mangan(III)-Ionen optional unter Verwendung einer Redox-Elektrode überwacht wird, wobei die Elektrolyse gestoppt wird, wenn der Mangan(III)-Gehalt den gewünschten Pegel erreicht; und/oder
weiterhin optional wobei, wenn das Verfahren den Schritt des Überwachens der Ansammlung von Mangan(III)-Ionen in der Lösung umfasst, die Ansammlung von Mangan(III)-Ionen optional durch Titrieren der Ätzlösung überwacht wird, wobei die Elektrolyse gestoppt wird, wenn der Mangan(III)-Gehalt den gewünschten Pegel erreicht; und/oder
weiterhin optional wobei, wenn das Verfahren den Schritt des Überwachens der Ansammlung von Mangan(III)-Ionen in der Lösung umfasst, das Verfahren weiterhin ein Überwachen der Konzentration von Mangan(II)-Ionen in der Lösung umfasst.

8. Verfahren nach Anspruch 5, das den Schritt eines periodischen Umkehrens des Stroms in der elektrolytischen Zelle umfasst, wodurch eine Ansammlung von Mangandioxid an der Anode verhindert wird.

9. Verfahren nach Anspruch 5, das weiterhin den Schritt eines Inkontaktbringens eines metallisierbaren Kunststoffs mit dem metastabilen Komplex für einen Zeitraum um Ätzen des metallisierbaren Kunststoffes umfasst,
optional wobei der metallisierbare Kunststoff Acrylnitril-Butadien-Styrol oder Acrylnitril-Butadien-Styrol/Polycarbonat umfasst und/oder
wobei vor dem Inkontaktbringen des metallisierbaren Kunststoffs mit dem metastabilen Komplex der metallisierbare Kunststoff mit einer Vorbehandlungszusammensetzung in Kontakt gebracht wird, um die Oberfläche des metallisierbaren Kunststoffs zu konditionieren, wobei die Vorbehandlungszusammensetzung ein Lösungsmittel umfasst, das aus der Gruppe bestehend aus Propylencarbonat, Gammabutyrolacton und Kombinationen davon ausgewählt ist, vorzugsweise wobei das Lösungsmittel Propylencarbonat umfasst,
optional wobei die Vorbehandlungslösung weiterhin eine organische Hydroxysäure umfasst, vorzugsweise wobei die organische Hydroxysäure aus der Gruppe bestehend aus Milchsäure, Glykolsäure, Glukonsäure und Kombinationen von einer oder mehreren der vorstehenden ausgewählt ist;
weiterhin optional wobei, wenn die Vorbehandlungslösung eine organische Hydroxysäure umfasst, die Vorbehandlungszusammensetzung bei einer Temperatur zwischen 20 und 70 °C gehalten wird und der metallisierbare Kunststoff mit der Vorbehandlungszusammensetzung für 2 bis 10 Minuten in Kontakt gebracht wird.

10. Verfahren nach Anspruch 5, wobei die Mangan(II)-Ionen von einer Verbindung abgeleitet sind, die aus der Gruppe bestehend aus Mangansulfat, Mangancarbonat und Manganhydroxid ausgewählt ist, und/oder
wobei die Lösung zusätzlich kolloidales Mangandioxid umfasst und/oder
wobei die Konzentration der Mangan(II)-Ionen in dem Elektrolyt zwischen 0,005 Mol und Sättigung liegt und/oder
wobei der Elektrolyt keinerlei Permanganat enthält.

11. Verfahren nach Anspruch 5, wobei die Kathode ein Material umfasst, das aus der Gruppe bestehend aus Platin, platiniertem Titan, Iridium-/Tantaloxid, Niob und Blei ausgewählt ist,
optional wobei die Kathode Blei umfasst und/oder wobei die Kathode platiniertes Titan oder Platin umfasst.

12. Verfahren nach Anspruch 5, wobei die Anodenstromdichte zwischen 0,1 und 0,4 A/dm² liegt und/oder
wobei die Temperatur des Elektrolyts zwischen 30 °C und 80 °C gehalten wird.

## Revendications

1. Cellule électrolytique comprenant :
une solution électrolyte comprenant des ions manganèse(III) et des ions manganèse(II) dans une solution comportant de l'acide sulfurique et un acide supplémentaire sélectionnés dans le groupe constitué d'acide méthane-sulfonique, méthane disulfonique et de combinaisons de ceux-ci, dans lequel la solution comporte une concentration d'au moins 8 M d'acide sulfurique;
une cathode en contact avec la solution électrolyte ; et
une anode en contact avec la solution électrolyte.

2. Cellule électrolytique selon la revendication 1, dans lequel la solution comprend éventuellement une concentration d'au moins 12 M d'acide sulfurique, et/ou
dans lequel la solution comprend une concentration de 1 M à 6 M d'acide méthane-sulfonique ou d'acide disulfonique, et/ou
dans lequel la solution comprend un rapport molaire de 9 à 15 d'acide sulfurique et une concentration de 1 M à 6 M d'acide méthane-sulfonique.

3. Cellule électrolytique selon la revendication 1, dans lequel une région de l'anode est plus étendue qu'une région de la cathode et/ou dans lequel l'anode comprend une matériau sélectionné dans le groupe constitué de carbone vitreux, de carbone vitreux réticulé, de fibres de carbone tissées, de plomb, d'alliage de plomb, de titane platiné, de platine, d'oxyde d'iridium/de tantale, de niobium, de diamant dopé au bore, et de combinaisons de l'un ou de plusieurs des éléments précédents, de préférence constitué de plomb ou d'alliage de plomb ;
dans lequel, quand l'anode comprend du plomb ou de l'alliage de plomb, la cellule électrolytique comporte aussi éventuellement un moyen permettant de surveiller la concentration de Mn(II) dans la solution.

4. Cellule électrolytique selon la revendication 1, dans lequel la cathode comprend un matériau sélectionné dans le groupe constitué de platine, de titane platiné, d'oxyde d'iridium/de tantale, de niobium et de plomb,
éventuellement dans lequel la cathode comporte du plomb ou
dans lequel la cathode comporte du titane platiné ou du platine.

5. Procédé d'oxydation électrochimique d'ions manganèse(II) en d'ions manganèse(III) comprenant les étapes consistant à :
fournir un électrolyte comportant une solution d'ions manganèse(II) dans une solution d'acide sulfurique à une concentration d'au moins 8 M, et un acide supplémentaire sélectionné dans le groupe constitué d'acide méthane-sulfonique, d'acide méthane-disulfonique et de combinaisons de ceux-ci dans une cellule électrolytique, dans lequel la cellule électrolytique comporte une anode et une cathode ;
appliquer un courant entre l'anode et la cathode ; et
oxyder l'électrolyte pour former des ions manganèse(III), dans lequel les ions manganèse(III) forment un complexe métastable.

6. Procédé selon la revendication 5, dans lequel l'électrolyte comprend une concentration de 1 M à 6 M d'acide méthane-sulfonique.

7. Procédé selon la revendication 5, dans lequel l'anode comporte du plomb ou de l'alliage de plomb,
éventuellement comprenant en outre l'étape consistant à surveiller la formation d'ions manganèse(III) dans la solution ;
en outre éventuellement dans lequel, quand le procédé comprend l'étape consistant à surveiller la formation d'ions manganèse(III) dans la solution, éventuellement pas plus de 50 % de la concentration originale d'ions manganèse(II) est oxydée en ions manganèse(III), de préférence pas plus de 25 % de la concentration originale d'ions manganèse(II) est oxydée en ions manganèse(III) ; et/ou
en outre éventuellement dans lequel, quand le procédé comprend l'étape consistant à surveiller la formation d'ions manganèse(III) dans la solution, la formation d'ions manganèse(III) est éventuellement surveillée en utilisant une électrode de potentiel redox, dans lequel l'électrolyse est arrêtée quand la teneur en manganèse(III) atteint le niveau désiré ; et/ou
en outre éventuellement dans lequel, quand le procédé comprend l'étape consistant à surveiller la formation d'ions manganèse(III) dans la solution, la formation d'ions manganèse(III) est éventuellement surveillée par titrage de la solution d'attaque, dans lequel l'électrolyse est arrêtée quand la teneur en manganèse(III) atteint le niveau désiré ; et/ou
en outre éventuellement dans lequel le procédé comprend l'étape consistant à surveiller la formation d'ions manganèse(III) dans la solution, le procédé consiste en outre à surveiller la concentration d'ions manganèse(II) dans la solution.

8. Procédé selon la revendication 5, comprenant l'étape consistant à périodiquement inverser le courant dans la cellule électrolytique, grâce auquel la formation de dioxyde de manganèse sur l'anode est évitée.

9. Procédé selon la revendication 5, comprenant en outre l'étape consistant à mettre en contact un plastique placable avec un complexe métastable pendant une certain temps pour attaquer le plastique placable,
éventuellement dans lequel le plastique placable est constitué de d'acrylonitrile-butadiène-styrène ou d'acrylonitrile-butadiène-styrène-polycarbonate, et/ou
dans lequel en amont de la mise en contact du plastique placable avec le complexe métastable, le plastique placable est mis en contact avec une composition de prétraitement pour conditionner la surface du plastique placable, la composition de prétraitement comportant un solvant sélectionné dans le groupe constitué de carbonate de propylène, de gamma-butyrolactone et de combinaisons de ceux-ci, de préférence dans lequel le solvant comprend du carbonate de propylène,
éventuellement dans lequel la solution de prétraitement comprend en outre un acide hydroxylé organique, de préférence dans lequel l'acide hydroxylé organique est sélectionné dans le groupe constitué d'acide lactique, d'acide glycolique, d'acide gluconique et de combinaisons de l'un ou de plusieurs des éléments précédents ;
en outre éventuellement dans lequel, quand la solution de prétraitement comprend de l'acide hydroxylé organique, la composition de prétraitement est maintenue à une température comprise entre 20 °C et 70 °C et le plastique placable est mis en contact avec la composition de prétraitement pendant une durée de 2 à 10 minutes.

10. Procédé selon la revendication 5, dans lequel les ions manganèse(II) proviennent d'un composé sélectionné dans le groupe constitué de sulfate de manganèse, de carbonate de manganèse et d'hydroxyde de manganèse, et/ou
dans lequel la solution comprend en supplément du dioxyde de manganèse colloïdal, et/ou
dans lequel la concentration d'ions manganèse(II) dans l'électrolyte est de 0,005 molaire à saturation, et/ou
dans lequel l'électrolyte ne contient aucun permanganate.

11. Procédé selon la revendication 5, dans lequel la cathode comporte un matériau constitué de platine, de titane platiné, d'oxyde d'iridium/de tantale, de niobium et de plomb,
éventuellement dans lequel la cathode comporte du plomb et/ou
dans lequel la cathode comporte du titane platiné ou du platine.

12. Procédé selon la revendication 5, dans lequel la densité du courant d'anode est de 0,1 à 0,4 A/dm², et ou
dans lequel la température de l'électrolyte est maintenue entre 30 °C et 80 °C.
